

C. S. BIRD.  
BUILDING MATERIAL.  
APPLICATION FILED AUG. 21, 1911.

1,181,827.

Patented May 2, 1916.

Fig. 1.



Fig. 2.



Fig. 3.



Witnesses:

Lucius P. Weymouth,  
M. J. M. Kay.

Inveterates:

Charles S. Bird  
By Henry J. Miller, Atty.

# UNITED STATES PATENT OFFICE.

CHARLES S. BIRD, OF WALPOLE, MASSACHUSETTS.

## BUILDING MATERIAL.

1,181,827.

Specification of Letters Patent. Patented May 2, 1916.

Application filed August 21, 1911. Serial No. 645,254.

*To all whom it may concern:*

Be it known that I, CHARLES S. BIRD, of Walpole, in the county of Norfolk and State of Massachusetts, have invented certain new and useful Improvements in Building Material, of which the following is a specification, reference being had to the accompanying drawings, forming part thereof.

This invention has reference to improvements in building material and particularly to roofing paper.

The object of the invention is so to construct building materials and particularly roofing paper having a layer of asphaltic or similar waterproof material provided with a coating of comparatively fine mineral particles that said surface may, in appearance, simulate a series of slates and, in addition, to more securely fix certain areas of said particles in place.

The invention consists in a sheet or strip of building material having a waterproof layer provided with a coating of particles adapted to mechanically protect said layer and having an overlying pattern of material in which said particles or certain groups or areas of said particles are embedded.

The invention also consists in the improved building material hereinafter described and claimed.

Figure 1, represents a plan view of the improved building material. Fig. 2, represents an enlarged sectional view taken on line 2—2, Fig. 1. Fig. 3, represents a similar view illustrating, approximately, the application of the additional surface coating of binding material.

Similar numerals of reference designate corresponding parts throughout.

In carrying this invention into practice it has been my main object to produce building material and particularly building paper having a more ornamental appearance than that heretofore constructed and at the same time to improve the wearing quality of the surface coating or of parts thereof. Building material of this nature has heretofore been constructed by taking a sheet or strip of paper and applying to one surface thereof a layer of viscous material preferably of an asphaltic or bituminous nature, portions of which were absorbed by the paper while the remainder formed a substantially water proof coating covering the paper. While the surface of this coating was still suffi-

ciently soft to be somewhat adhesive fine mineral particles have been applied thereto and have adhered to such coating in sufficient quantities to form a surface coating to 60 mechanically protect the surface of the waterproof material from the action of the weather. This unbroken surface of the protective coating, with the straight edges of the strip has been monotonous in appearance and has militated against the use of the material on buildings of the higher class such as dwellings. Various attempts have been made to produce an ornamental effect with such material without much success as 70 such attempts have resulted in reducing the life of the material by removing some portions thereof, leaving raw edges.

In constructing my improved building material I take a sheet or strip 5 of paper or other suitable material adapted to be used as a base or backing and to such base I apply water proofing or water resisting material in a semifluid or plastic condition to form the layer 6 which adheres to the base 5, and preferably, is partially absorbed by such base. The material of said layer 6 is preferably of such nature that its surface remains comparatively soft for a period after its application sufficient to permit the particles 7, 7 now applied thereto, to adhere to such surface while the greater portions of such particles 7, 7 extend outward from said layer 6 and mechanically protect said surface from the weather. The 90 material thus constructed has the appearance of a sanded surface of substantially the color of the particles 7, 7 which of course may be artificially colored prior to their application to the layer 6. I now take 95 fluid or semifluid material substantially of the nature of the material of the layer 6 and of a color contrasting with the general color effect of the combined particles 7, 7 and apply such material in areas, lines or 100 stripes 8, 8 of comparative thickness, in any predetermined pattern to the surface formed by the particles 7, 7 whereby said material of the areas 8, 8 forms a binder for the particles 7, 7 which it covers and, to some extent unites with the layer 6, while the contrasting color of such material 8, 8 forms a design or pattern on the outer surface of the strip by covering certain of said particles, groups or areas of said particles. It 110 will thus be seen that the layer 6 is protected throughout by the coating of par-

ticles 7, 7 while the appearance of the material is greatly improved, and such of said particles 7, 7 as are embedded, in and covered by the overlying material 8, 8 are more secure than heretofore.

While I prefer to make use of asphaltic material for layer 6 and for the overlay 8, 8 I do not limit myself to the use of such material. The particles 7, 7 may be 10 grains of sand, soapstone or any other natural or artificial particles adapted for the purpose herein described.

While I have herein attempted to show my improved building material by drawings it is evident that such showing of material can be only approximate and I do not wish to limit myself to the exact showing in 15 said drawings.

I prefer to apply the material forming 20 the overlay pattern 8, 8 in such a manner of such consistency and condition that it will be readily received between the particles 7, 7 and, to some extent, will unite with material of the layer 6.

Having thus described my invention, I 25 claim as new and desire to secure by Letters Patent.

1. Building material of the nature described comprising a sheet having a continuous coating of comparatively fine particles and an overlay pattern of asphaltic material covering areas of said particles.

2. Building material of the nature described comprising a base having a protective coating of substantially water-proof material, and an overlay pattern of substantially similar material dividing said protective coating into areas, lines or stripes, said protective coating in said

areas, lines or stripes having fine particles 40 adhering thereto.

3. Building material of the nature described comprising a base having a coating of water-proof material, an overlay pattern of substantially similar material to 45 vary the thickness of said coating, and a substantially continuous layer of fine particles extending practically throughout the surface plane of said waterproof material and embedded to some extent therein. 50

4. Building material of the nature described comprising a base having a layer of waterproof material, an overlay pattern of similar material, and a coating of fine particles secured by adhesion to said layer, 55 areas of said particles being embedded in and covered by said overlay, substantially as described.

5. Building material of the nature described comprising a base having an asphaltic layer furnished with a coating of fine mineral particles, and an overlay pattern of comparatively thick plastic material in which certain areas of said particles are 60 embedded and covered, substantially as described.

6. Prepared roofing comprising a sheet of fibrous material impregnated and coated with a waterproof material, said coating being varied in thickness in various fields, 70 a coating of granular grit partially embedded in said coating in the fields of least thickness, and a similar coating completely embedded in the fields of greater thickness.

CHARLES S. BIRD.

Witnesses:

H. H. MILLER,  
HENRY J. MILLER.